

Nov. 17, 1925.

1,562,384

C. M. TAYLOR

FLOOR COVERING AND PROCESS OF MAKING SAME

Original Filed Jan. 10, 1922

*FIG. 1.*



*FIG. 2.*



Inventor

C. Marshall Taylor.

By Prentiss, Stone & Boyden.  
Attorneys.

Patented Nov. 17, 1925.

1,562,384

# UNITED STATES PATENT OFFICE.

CALEB MARSHALL TAYLOR, OF ELIZABETH, NEW JERSEY.

## FLOOR COVERING AND PROCESS OF MAKING SAME.

Application filed January 10, 1922, Serial No. 528,300. Renewed September 1, 1925.

To all whom it may concern:

Be it known that I, CALEB MARSHALL TAYLOR, a citizen of the United States, residing at Elizabeth, in the county of Union and

5 State of New Jersey, have invented certain new and useful Improvements in Floor Coverings and Processes of Making Same, of which the following is a specification.

This invention relates to floor coverings 10 and to a process of making the same.

The floor covering provided is of that type known as felt base floor coverings and particularly such materials in which an asphalt or bitumen impregnated base is used.

15 The invention is also peculiarly adapted for use in combination with all floor coverings in which either the wear surface or the opposite face is formed of paint or other material containing linseed oil or other oil, 20 or any material subject to saponification or removable under the action of soap and the usual floor cleaning materials.

25 Bitumen impregnated felt base floor coverings may be recognized by the main dark body which is particularly evident when the material is cut. The felt of such bases may be made from rags or from paper or any cellulose material, or from a mixture of such materials, thoroughly impregnated with 30 asphalt or tar or some suitable bituminous material. When used as a supporting base for floor covering it is the usual practice to coat the bitumen impregnated base with a layer of paint which is known as a sealing 35 coat and often to apply various painted designs, all of which may be applied in any convenient manner. Also, a coat of paint is applied to the opposite or under surface of the impregnated base to cover the dark 40 and unsightly bitumen impregnated base.

45 For the manufacture of such bitumen impregnated bases it has been found that the wear paint and the decorative paint may become discolored due in part to the inherent nature of the bitumen of the base. Also in 50 drying the paint coats it is necessary to dry at relatively low temperatures and for a correspondingly long period, often as long as four or five days. A higher temperature and more rapid drying would tend to liquefy the bitumen and delay proper drying of the paint and also discolor the paint due to the release of materials from the base.

Thus a baking temperature of 175° F. or more, such as is desirable for treating the 55 paint coats, is not advisable in the usual drying of such coated bases.

After the present known product is completed it is usually necessary to place paper between adjacent surfaces when the material 60 is rolled or stacked in layers to prevent the adjacent painted surfaces from adhering. It is well known that all such painted surfaces, and also that surface of the material known as linoleum is worn away by the use of soap 65 and water because of saponification by such cleaning materials on the oils in the paint and linoleum.

The present invention makes it possible to use the relatively inexpensive bitumen 70 impregnated felt base without discoloration of the wear or decorative paint coats, and results not only in reducing the time of drying the paint coats to a much shorter length of time, but makes it possible to use 75 a higher drying temperature for the paint and to produce a more lasting finish on the painted surface.

In producing the impregnated felt base of this invention, the usual rolls of asphalt 80 or bitumen impregnated felt may be used. A solution is prepared of a mixture of nitro-cellulose and a solvent therefor. Preferably the desired quantity of a semi-drying or drying vegetable oil is added to the mixture 85 as a softening medium. The solution is applied to one or both surfaces of the impregnated base as a sealing coat by any well known coating process. The solution thus applied is quickly dried on the base. A suitable drying temperature is approximately 90 140° F. The impregnated base is thus provided with an impervious film which may be used wherever an ordinary bitumen impregnated base would not have been acceptable 95 before on account of the sticky, tar-like nature of its materials.

One or more paint coats are then applied and the structure baked at a temperature of 175° F. or more to dry the paint and provide the desired wearing surface. The coating of impervious pyroxylin over the felt base prevents the dark material from the base from discoloring the paint.

If desired the product thus prepared may 105 be coated with an outer transparent coating.

2 as described and claimed in my copending application Serial No. 528,301.

In the accompanying drawing:

5 Figure 1 illustrates an enlarged sectional view of a felt base 1 having an upper coating 2 of the pyroxylin solution and if desired an under coating 3 of the same material. The invention thus far is described and claimed in my copending application 10 Serial No. 528,298. A paint coat 4 is applied on top of the surface 2 and an outer decorative paint coat is indicated at 5. Figure 2 is a plan view of the same.

15 Other cellulose esters than nitrocellulose, such as acetyl cellulose, may be used.

20 One satisfactory mixture for the solution for the coating may be made by using 12 parts by weight of nitrocotton, and 88 parts by weight of a solvent mixture which may be composed of 35 per cent of acetone oil and 65 per cent of such a diluent as solvent naphtha, xylol, toluol, or benzol. Any well known working formula may be used for combining such a mixture of drying or semi- 25 drying vegetable oil and nitrocotton. To such a mixture may be added 12 parts by weight of linseed oil or other semi-drying or drying vegetable oil. 12 parts by weight of resin, such as cumaron, kauri or camphor 30 may be incorporated in the mixture to advantage.

35 To the cellulose mixture may be added a pigment color in any desired shade and amount. This results in a tinted film formed from a solution, as contrasted with a plastic material, in which the same shade extends through the thickness of the film, a feature which is new in such cellulose coatings and particularly in floor coverings. This is to be contrasted to the tinted pyroxylin plastics 40 such as are applied by plastic working apparatus.

45 The sealing coat increases the tensile strength of the bitumen saturated base about 10 per cent. The sealing coat may be advantageously applied to the impregnated felt base at the felt impregnating factory and before shipment. The material possesses good wearing qualities whether it is considered as an underneath coating or as an 50 upper wear coat. A further advantage of the use of the sealing coat, particularly the coat on the back or under surface, is derived from the fact that it prevents the discoloring 55 of the upper face of the finished goods when these are rolled up, or otherwise come in contact with each other. The sealing coat which is applied to the back may likewise carry enough pigment to give the desired 60 shade of color.

I claim:

65 1. A floor covering comprising a bitumen impregnated felt base, an imperforate coating of a cellulose ester on said base, and a coating of paint on said cellulose ester.

2. A floor covering comprising a bitumen impregnated felt base, an imperforate coating of a mixture of a cellulose ester and a softening medium on said base, and a coating of paint on said cellulose ester. 70

3. A floor covering comprising a bitumen impregnated felt base, an imperforate coating of nitrocellulose on said base, and a coating of paint on said nitrocellulose coating. 75

4. A floor covering comprising a bitumen impregnated felt base, an imperforate coating of a mixture of nitrocellulose and a softening medium on said base, and a coating of paint on said nitrocellulose coating. 80

5. A floor covering comprising a bitumen 85 impregnated felt base, an imperforate coating of a mixture of nitrocellulose and a resin on said base, and a coating of paint on said nitrocellulose coating.

6. A floor covering comprising a bitumen impregnated felt base, an imperforate coating of a mixture of nitrocellulose, a resin, and a vegetable oil, and a coating of paint on said nitrocellulose coating. 85

7. A floor covering comprising a bitumen 90 impregnated felt base, an imperforate coating of a mixture of cellulose ester, and a resin on said base, and a coating of paint on said cellulose ester coating.

8. A floor covering comprising a bitumen 95 impregnated felt base, an imperforate coating of a mixture of cellulose ester, a resin, and a vegetable oil, and a coating of paint on said cellulose ester coating.

9. A floor covering comprising a bitumen 100 impregnated base, an imperforate coating of a cellulose ester on said base, and a coating of paint on said cellulose ester.

10. A floor covering comprising a bitumen 105 impregnated base, an imperforate coating of a cellulose ester on said base, and a baked coating of paint on said cellulose ester.

11. A floor covering comprising a bitumen 110 impregnated base, an imperforate coating of nitrocellulose on said base, and a coating of 115 paint on said nitrocellulose coat.

12. The process of making floor coverings which comprises coating a bitumen impregnated felt base with a solution of a cellulose ester, drying said solution, and applying to 120 said dried surface a coat of paint.

13. The process of making floor coverings which comprises coating a bitumen impregnated felt base with a solution of a cellulose ester, drying said solution, applying to said 125 dried surface a coat of paint, and subjecting the base and coatings to a temperature of approximately 140° F.

14. The process of making floor coverings which comprises coating a bitumen impregnated felt base with a mixture in solution of a cellulose ester and a softening medium, drying said solution, applying to said dried surface a coat of paint, and drying the paint 130 coat.

15. The process of making floor coverings which comprises coating a bitumen impregnated felt base with a solution of a cellulose ester, which solution contains approximately 12 parts by weight of the cellulose ester and 88 parts of solvent, drying said solution, and applying to said dried surface a coat of paint.
16. The process of making floor coverings which comprises coating a bitumen impregnated felt base with a mixture in solution of a cellulose ester and a softening medium, which solution contains approximately 12 parts by weight of cellulose ester, 88 parts of solvent, and 12 parts of softening medium, drying said solution, and applying to said dried surface a coat of paint.
17. The process of making floor coverings which comprises coating a bitumen impregnated felt base with a mixture in solution of a cellulose ester, which solution contains approximately 12 parts by weight of cellulose ester, 88 parts of a solvent thereof, and 12 parts of a resin, drying said solution, and applying to said dried surface a coat of paint.
18. The process of making floor coverings which comprises coating a bitumen impregnated felt base with a mixture in solution of a cellulose ester, which solution contains approximately 12 parts by weight of a cellulose ester, 88 parts of a solvent thereof, 12 parts of a resin, and 12 parts of a vegetable oil, drying said solution, and applying to said dried surface a coat of paint.
19. The process of making floor coverings which comprises coating a bitumen impregnated felt base with a solution of nitrocellulose, drying said solution, and applying to said dried surface a coat of paint.
20. The process of making floor coverings which comprises coating a bitumen impregnated felt base with a solution of nitrocellulose, drying said solution, applying to said dried surface a coat of paint and subjecting the base and coatings to a temperature of approximately 140° F.
21. The process of making floor coverings which comprises coating a bitumen impregnated felt base with a mixture in solution of nitrocellulose and a softening medium, drying said solution, applying to said dried surface a coat of paint, and drying the paint coat.
22. The process of making floor coverings which comprises coating a bitumen impregnated felt base with a solution of nitrocellulose, which solution contains approximately 12 parts by weight of the nitrocellulose and 88 parts of solvent drying said solution, and applying to said dried surface a coat of paint.
23. The process of making floor coverings which comprises coating a bitumen impregnated felt base with a mixture in solution of nitrocellulose and a softening medium, which solution contains approximately 12 parts by weight of nitrocellulose, 88 parts of solvent, and 12 parts of softening medium, drying said solution, and applying to said dried surface a coat of paint.
24. The process of making floor coverings which comprises coating a bitumen impregnated base with a solution of nitrocellulose, drying said solution, and applying to said dried surface a coat of paint.
25. The process of making floor coverings which comprises coating a bitumen impregnated base with a solution of nitrocellulose, drying said solution, applying to said dried surface a coat of paint, and subjecting said base and coatings to a temperature of approximately 140° F.
26. The process of making floor coverings which comprises coating a bitumen impregnated base with a solution of a cellulose ester, drying said solution, applying to said dried surface a coat of paint, and subjecting said base and coatings to a baking temperature to harden the surface of the paint coat.
27. A smooth surface floor covering comprising a porous base impregnated with a flexible bitumen saturant filling material, an imperforate coating of a film of a cellulose ester on said base, and a coating of paint on said cellulose ester film.
28. A smooth surface floor covering comprising a porous fibrous base impregnated throughout with a flexible bitumen saturant filling material, an imperforate coating of a film of a cellulose ester on said base, and a coating of paint on said cellulose ester film.
- In testimony whereof I affix my signature.  
CALEB MARSHALL TAYLOR.